

Nov. 3, 1936.

F. RITTERSHAUSEN

2,059,746

HOMOGENEOUS ARMOR PLATE

Filed Oct. 27, 1932



Inventor:  
Fritz Rittershausen  
By Knight Bros.  
His Atlys.

## UNITED STATES PATENT OFFICE

2,059,746

## HOMOGENEOUS ARMOR PLATE

Fritz Rittershausen, Essen, Germany, assignor to  
 Fried. Krupp Aktiengesellschaft, Essen-on-  
 the-Ruhr, Germany

Application October 27, 1932, Serial No. 639,881  
 In Germany December 15, 1931

5 Claims. (Cl. 148—21.5)

My invention relates to homogeneous armor plates. By the term "homogenous armor plate", which here comprises also roof or deck plates, is meant a plate manufactured from a steel alloy and showing a uniform texture on its entire cross section, that is a plate which for example is not hardened on one side or cemented and hardened.

The known homogenous armor plates of highest quality are made from steel alloys which contain about 0.25 to 0.35% carbon, 3 to 5% nickel, 1 to 1.8% chromium and sometimes up to 0.5% molybdenum, the addition of molybdenum serving in these known armor plates to facilitate the heat treatment and to avoid the danger of tempering brittleness. The nickel is considered as the bearer of the toughness, and since great value is attached to very high toughness, the nickel content generally is fixed at 3.5% at least.

Exhaustive researches have now shown that the toughness of armor plates and thus their resistance to striking projectiles, especially to oblique fire, and their safety against being pierced by bursting shells, is not only not reduced but can even be considerably improved by reducing the nickel content to about 3% or less, provided the carbon content is kept on about 0.12 to 0.42% and the chromium content on 2 to about 3.75%, and molybdenum is present in the alloy in an amount from 0.2 to 1%, while the total of chromium and nickel should not be higher than indicated by the curve A of the accompanying drawing. It is of particular advantage so to determine the composition of the armor plates that it comes within the hatched area B of the drawing, wherein the compositions situated in the upper part thereof and containing higher totals of chromium and nickel are especially suited for thicker plates, whilst for

plates of smaller thickness the compositions coming within the lower part of the area B are especially fit. The effect of the molybdenum may be obtained also by about 1.5 to 3 times as much tungsten. In certain cases the nickel may be entirely dispensed with. The cause of the superiority explained above of the proposed composition of armor plates is to be seen, in the opinion of the inventor, in the feature that in heating the plates the  $A_{ci}$  critical point, which must not be exceeded in the heat treatment following the hardening treatment, is substantially higher in the new armor plates than with the known plates richer in nickel, so that it is possible to reheat the new plates even at temperatures up to about 700° C. This higher reheating

treatment, however, which cannot be employed with the known plates, richer in nickel and poorer in chromium, imparts to the plates a substantially higher toughness and thus a substantially improved resistance to being damaged by projectiles. For heat treated armor plates, that is plates of the above composition and hardened and reheated in the above-described manner show a notch toughness of about 35 mkg/cm<sup>2</sup> (normal Charpy test) and a tensile strength of about 70 kg/mm<sup>2</sup>.

The same high toughness, but with a slightly lower tensile strength, can be obtained, by virtue of the high critical point, even by a simple heating at temperatures up to about 750° C.

The armor plates forming the subject-matter of the present invention are distinguished for the advantage of having a substantially higher resistance to projectiles and of being manufactured at substantially lower costs, owing to the nickel content being smaller or dispensed with altogether.

Particularly advantageous examples of the armor plates according to the invention are the following:

1. Homogeneous armor plate of 70 mm. thickness, containing about 0.2% carbon, 2.4% chromium, 0.4% molybdenum, no nickel.

2. Homogeneous armor plate of 100 mm. thickness, containing about 0.19% carbon, 2.3% chromium, 0.4% molybdenum and 1.5% nickel.

3. Homogeneous armor plate of 80 mm. thickness, containing about 0.32% carbon, 2.6% chromium, 0.6% nickel, and 0.38% molybdenum.

4. Homogeneous armor plate of 120 mm. thickness, containing about 0.39% carbon, 2.5% chromium, 1.8% nickel and 0.45% molybdenum.

What I claim and desire to secure by Letters Patent is:—

1. The process of heat treating a homogeneous armor plate made from a steel alloy containing about 0.12 to 0.42% carbon, about 2 to 3.75% chromium, an appreciable amount of nickel not over about 3%, and metal selected from the group molybdenum, tungsten in the proportion 0.2 to 1% molybdenum, 0.3 to 3% tungsten, the remainder substantially all iron, the total of chromium and nickel referred to the carbon content being not higher than indicated by the curve A of the drawing, which process consists in hardening the plates throughout by a uniform heat treatment and reheating them at a temperature of about 700° C.

2. The process of heat treating a homogeneous armor plate made from a steel alloy containing

- about 0.12 to 0.42% carbon, about 2 to 3.75% chromium, an appreciable amount of nickel not over about 3%, and metal selected from the group molybdenum, tungsten in the proportion 0.2 to 5 1% molybdenum, 0.3 to 3% tungsten, the remainder substantially all iron, the carbon and chromium plus nickel content of which comes within the area B of the drawing, which consists in hardening the plates throughout by a uniform heat treatment and reheating them at a temperature of about 700° C.
3. Homogeneous armor plate made from a steel alloy containing about 0.12 to 0.42% carbon, about 2 to 3.75% chromium, an appreciable amount of 15 nickel not over about 3%, and metal selected from the group molybdenum, tungsten in the proportion 0.2 to 1% molybdenum, 0.3 to 3% tungsten, the remainder substantially all iron, the total of chromium and nickel, referred to the carbon 20 content, being not higher than indicated by the curve A of the drawing, said steel alloy being in a substantially homogeneous hard and tough condition throughout resulting from a hardening heat treatment followed by reheating to about 25 700° C.
4. Homogeneous armor plate made from a steel alloy containing about 0.12 to 0.42% carbon, about 2 to 3.75% chromium, an appreciable

amount of nickel not over about 3%, and about 0.2 to 1% molybdenum, the total of chromium and nickel, referred to the carbon content, being not higher than indicated by the curve A of the drawing, said steel alloy being in a substantially homogeneous hard and tough condition throughout resulting from a hardening heat treatment followed by reheating to about 700° C., said plate being characterized by a particularly high resistance to penetration by projectiles.

5. Homogeneous armor plate made from a steel alloy containing about 0.12 to 0.42% carbon, about 2 to 3.75% chromium, an appreciable amount of nickel not over about 3%, and metal selected from the group molybdenum, tungsten in 15 1% molybdenum, 0.3 to 3% tungsten, the remainder substantially all iron, the nickel content being at a figure between the limits stated determined according to a direct ratio between thickness of the armor plate and nickel 20 content, the total of chromium and nickel, referred to the carbon content, being not higher than indicated by the curve A of the drawing, said steel alloy being in a substantially homogeneous hard and tough condition throughout resulting 25 from a hardening heat treatment followed by reheating to about 700° C.

FRITZ RITTERSHAUSEN.